

June 6, 1944.

E. E. JELLEY ET AL

2,350,764

PHOTOGRAPHIC SCREENING LAYER

Filed Feb. 5, 1943



Edwin E. Jelley  
Paul W. Vittum  
INVENTORS

BY *Walter M. Purvis*  
*R. Frank Smith*  
ATTORNEYS

## UNITED STATES PATENT OFFICE

2,350,764

## PHOTOGRAPHIC SCREENING LAYER

Edwin E. Jelley and Paul W. Vittum, Rochester,  
N. Y., assignors to Eastman Kodak Company,  
Rochester, N. Y., a corporation of New Jersey

Application February 5, 1943, Serial No. 474,836

8 Claims. (Cl. 95—2)

This invention relates to photographic elements, and more particularly to such elements carrying screening material either in the emulsion layer or in a separate layer.

It is known that the amount of light which reaches a sensitive photographic element may be reduced or restricted to light of a definite color by the use of screening layers coated over the sensitive element. Numerous screening materials have been proposed among which are Tartrazine, Naphthol Yellow, and Quinoline Yellow. These dyes have the undesirable property of desensitizing cyanine sensitized emulsions and, therefore, are unsuitable for incorporation in emulsions which have been color-sensitized by cyanine dyes. Certain dyes and filter materials hitherto used have the additional undesirable property of diffusing or wandering from the layer in which they are incorporated. When it is desirable to coat a layer of sensitive emulsion or plain gelatin containing a dye or screening material adjacent to another layer which is to contain either a definite dye or no dye at all, it is essential that there be no wandering of the dye from layer to layer during or after coating; and when the layer in which the dye is incorporated is light sensitive, it is further essential that the dye does not desensitize the emulsion. The difficulties have been especially noticeable in yellow dyes.

The principal object of the present invention is to provide yellow filter materials which do not wander from the layer in which they are incorporated, which do not desensitize light-sensitive photographic emulsions and have the desired spectral absorptions.

The objects of the invention are accomplished by dispersing a metal salt of an osazone derivative of dihydroxy tartaric acid in a layer of a light-transmitting colloidal film-forming material.

The metal salts which our invention contemplates are those having the formula



The metal salts effective for our purpose have

the above formula wherein R is an aryl group as, for example, phenyl m-tolyl, p-carboxyl phenyl, p-nitrophenyl, 2,4-dinitrophenyl, p-(p-tert. butyl phenoxy) phenyl, naphthyl and substituted naphthyl, and M is either calcium, barium, strontium, or magnesium. These salts are removable from water-permeable layers in which they are incorporated, by means of alkaline photographic processing solutions.

10 For the carrier material for the filter layer, whether it be a layer of a multilayer film or a layer such as a Wratten filter layer containing the above compound, may be used gelatin, cellulose esters and natural or synthetic resins, especially gelatin and water-permeable cellulose esters and resins where the layer must be permeable to alkaline photographic processing solutions in order to remove the metal salt from the layer after it has served its purpose in screening underlying sensitive layers.

15 The following table gives the colors of representative calcium salts of the compounds of our invention where R in the above formula is a phenyl or substituted phenyl group.

|    | R                               | Color          |
|----|---------------------------------|----------------|
| 30 | Phenyl                          | Yellow.        |
|    | m-Tolyl                         | Yellow-orange. |
|    | p-Carboxyl phenyl               | Yellow.        |
|    | p-Nitrophenyl                   | Orange.        |
|    | 2,4-dinitrophenyl               | Orange-red.    |
|    | p-(p-tert. Butyl phenoxy)phenyl | Yellow.        |

20 The preparation of salts of dihydroxy tartaric acid phenyl osazone is described in Berichte der Deutschen Chem. Gesellschaft, vol. 20, 1887, pages 836-838. The preparation of salts of dihydroxy tartaric acid p-nitrophenyl osazone is described by Gnehm und Benda in Annalen der Chemie, vol. 299, 1898, pages 104-106. The m-tolyl, p-carboxyl phenyl, and 2,4-dinitrophenyl derivatives are prepared similarly using m-tolyl hydrazine, p-carboxyl phenyl hydrazine or 2,4-dinitro hydrazine respectively as the starting materials, in place of the phenyl hydrazine or p-nitrophenyl hydrazine used in the methods of the references. In preparing the p-(p-tertiary butyl phenoxy) phenyl derivative, the corresponding hydrazine is employed. The

preparation of this hydrazine is described in British Patent 547,064.

The figure of the accompanying drawing shows in enlarged cross-sectional view a multilayer color film provided with a filter layer of composition contemplated by our invention.

In the figure of the drawing the support 10 of cellulose ester or other suitable material such as glass or paper carries the red, green and blue sensitive emulsion layers 11, 13, and 15, sensitized if desired by cyanine dyes, emulsion layers 11 and 13 being separated by a clear gelatin layer 12 and emulsion layers 13 and 15 by the yellow filter layer 14 of the invention, composed of a metal salt of one of the osazone derivatives of dihydroxy tartaric acid of formula shown previously. Thus, during exposure of the sensitive photographic element the screening layer 14 prevents passage of blue light from the top of the film to emulsion layers 11 and 13 which have inherent blue sensitivity in addition to conferred red and green sensitivity, respectively.

The following example is representative of the methods we use for incorporating the metal salts of the invention into layers of colloidal film-forming material.

A solution is made of 0.8 gram of sodium dihydroxy tartrate phenyl osazone in 8 cc. of distilled water and 20 cc. of 95 per cent ethyl alcohol. This is added to 50 cc. of a melted 10 per cent solution of de-ashed gelatin, and to this mixture is added rapidly a solution of 0.8 gram of calcium acetate (monohydrate) in 16 cc. of distilled water. The calcium osazone salt forms immediate and after coating the solution on a suitable surface and drying, there is obtained an intensely yellow colored layer in which the metal salt is substantially non-diffusing. The calcium salt of dihydroxy tartaric acid phenyl osazone prepared in the manner described by reaction of the sodium salt with a soluble calcium salt, was given the usual spectral absorption test and it was found that for wavelengths from about 520 mu to 460 mu the optical density varied from 0.36 to 2.4 falling off slightly at shorter wavelengths. The metal salts of the other aryl osazones have similar absorption curves but may be shifted depending on the color of the salt. We have compared the absorption curves of the compounds of the invention with those of other osazones and yellow filter materials and have found that our compounds absorb more completely in the blue region of the spectrum, as a result of which they are more satisfactory for use in color photography. For example, the sodium salt of glucose phenyl osazone-p,p'-dicarboxylate has an absorption curve showing that the compound has substantially no absorption at wavelengths longer than 460 mu.

As is apparent, the above solution of the colored salt when employed for coating a filter layer such as layer 14 of the drawing, is coated in a known manner on the green-sensitive emulsion layer 13 before coating the blue-sensitive emulsion layer 15 thereon. Other osazones and metal salts thereof contemplated by our invention are incorporated in a layer of gelatin or similar material in a similar manner. In case it is desired to incorporate the filter material in one of the emulsion layers, such as the blue-sensitive emulsion layer 15 of the multilayer film shown in the drawing, and this procedure and the film obtained thereby is considered to be a part of our invention, the metal salt is formed as above-

described in gelatin solution and added to the blue-sensitive emulsion before coating, or if desired, the metal salt may be formed in the sensitive emulsion.

5 Herein, and in the appended claims where we state that our invention includes a photographic element comprising a support having thereon a plurality of light-sensitive emulsion layers sensitive to different regions of the spectrum and a dispersion of a metal salt of formula given above, in colloidal film-forming material, we would have it understood that this includes incorporating the metal salt either in a separate layer of a multilayer film or in one of the emulsion layers thereof.

10 It is to be understood that our invention may be used in other ways not herein specifically mentioned and that we are to be limited only by the scope of the appended claims.

15 What we claim is:

20 1. A photographic element comprising a support having thereon at least one light-sensitive emulsion layer, and a dispersion of a metal salt having the formula



25 where R is an aryl group and M is a bivalent metal selected from the group consisting of calcium, barium, strontium, and magnesium, in light-transmitting colloidal film-forming material.

30 2. A photographic element comprising a support having thereon a plurality of light-sensitive emulsion layers sensitized to different regions of the spectrum, and having over one of said emulsion layers a layer of a dispersion of a metal salt having the formula



35 where R is an aryl group and M is a bivalent metal selected from the group consisting of calcium, barium, strontium, and magnesium, in light-transmitting colloidal film-forming material.

40 3. A photographic element comprising a support having thereon a plurality of light-sensitive emulsion layers sensitive to different regions of the spectrum, and over one of said emulsion layers a layer of a dispersion of a metal salt having the formula



45 where R is an aryl group and M is barium, in light-transmitting colloidal film-forming material.

50 4. A photographic element comprising a support having thereon a plurality of light-sensitive emulsion layers sensitive to different regions of the spectrum, and over one of said emulsion layers a layer of a dispersion of a metal salt having the formula



55 where R is a phenyl group and M is barium, in light-transmitting colloidal film-forming material.

60 5. A photographic element comprising a sup-

port having thereon a plurality of light-sensitive emulsion layers sensitive to different regions of the spectrum, and over one of said emulsion layers a layer of a dispersion of a metal salt having the formula



where R is an aryl group and M is calcium, 10 in light-transmitting colloidal film-forming material.

6. A photographic element comprising a support having thereon a plurality of light-sensitive emulsion layers sensitive to different regions of the spectrum, and over one of said emulsion layers a layer of a dispersion of a metal salt having the formula



where R is a phenyl group and M is calcium, in light-transmitting colloidal film-forming material.

7. A photographic element comprising a support having thereon a plurality of light-sensitive

emulsion layers sensitive to different regions of the spectrum, and over one of said emulsion layers a layer of a dispersion of a metal salt having the formula

5



where R is an aryl group and M is magnesium, in light-transmitting colloidal film-forming material.

8. A photographic element comprising a support having thereon a plurality of light-sensitive emulsion layers sensitive to different regions of the spectrum, and over one of said emulsion layers a layer of a dispersion of a metal salt having the formula

20



where R is a naphthyl group and M is magnesium, in light-transmitting colloidal film-forming material.

25

EDWIN E. JELLEY,  
PAUL W. VITTRUM.